

## UNITED STATES PATENT OFFICE

2,079,035

## PROCESS OF REFINING PETROLEUM

Theodor A. Petry, Woodbury, N. J., assignor to  
Socony-Vacuum Oil Company, Incorporated,  
New York, N. Y., a corporation of New York

No Drawing. Application September 10, 1935,  
Serial No. 39,938

8 Claims. (Cl. 196—13)

This invention relates to the refining of petroleum, and has to do particularly with the refining of the relatively viscous petroleum fractions to produce lubricating oil of good quality.

5 One object of the invention is to provide a process of refining petroleum lubricant stocks which is applicable generally to the treatment of any petroleum lubricant stock, including crude petroleum, distillation residues such as long 10 residuum or heavier residues, and in general any petroleum lubricant oil stock which contains fractions of good lubricating oil value but which also contains asphaltic matter and/or wax and naphthenic substances, to produce therefrom a refined 15 lubricating oil of high quality having high viscosity index, low carbon residue, and desired pour point.

It is a further object of the invention to provide a new solvent refining agent for extracting naphthenic substances and a process for refining petroleum stocks by means of this agent, this 20 solvent refining process being applicable to petroleum lubricant oil stocks generally but being preferably used in the refining of stocks which already have been treated to remove wax or asphaltic matter, or both.

25 Viscosity index is a numerical index, referred to an arbitrary scale, as proposed by Dean and Davis, "Chemical and Metallurgical Engineering", 36-618 (1929), and refers to the rate at which the viscosity of the oil decreases with increase in temperature. Pennsylvania base lubricants of present manufacture have a viscosity index of around 95 to 100, coastal naphthenic base lubricants have viscosity indices of about 0 to 20, and various Mid-Continent mixed base lubricants 30 range in between these values. It is possible for the viscosity index to be numerically less than 0 or more than 100. The higher index numbers indicate a greater resistance to loss of viscosity 35 with rise of temperature. In the present terminology of the art, the rapidly thinning constituents are spoken of as naphthenic, and the more slowly thinning constituents are spoken of as paraffinic. In this sense only, and not in a rigorous 40 chemical sense, the terms naphthenic and paraffinic are used herein.

The viscosity-gravity constant, proposed by Hill and Coates, Ind. & Eng. Chem. 1928, page 641 is 45 also a valuable indication of the "paraffinic" nature of an oil fraction as *v-g-c* value indicates increasing freedom from constituents highly naphthenic with decrease in numerical value of the constant. The *v-g-c* or viscosity-gravity- 50 constant for present day lubricants of Pennsyl-

vania origin is around 0.800 to 0.830 with lubricants from other sources ranging up to 0.900.

Carbon residue is the amount of weighed residue left when a given weight of oil is burned under certain specified conditions fully set forth in Bureau of Mines Technical Paper 323B, Method 500.12, commonly known as the Conradson carbon residue test. The result is expressed in per cent of residue and is indicative of carbon-forming and decomposition tendencies of the oil 10 when heated, an oil having a lower percentage of residue being one more able to endure under conditions of field performance.

Pour point, as referred to herein, shall mean the determination of pour point described in 15 A. S. T. M. Method D 97—33.

This invention has specifically to do with a solvent refining method, where a solvent reagent is used to extract naphthenic constituents of low viscosity index; etc., from the oil, and is especially directed to the use of a particular solvent 20 of that general class.

This invention has for an object the use of benzylamine as a solvent refining reagent capable of improving lubricating oils by separating from the petroleum lubricant stock constituents having undesirable characteristics; e. g. naphthenic 25 substituents. Benzylamine is the amine corresponding with benzyl alcohol, having the structural formula



30 That is, it is a primary amine with the amine group in the side chain. Chemically, it partakes more of the nature of methylamine than of that of aniline. This compound has been found to be possessed of a particularly high solvent power 35 when used in the treatment of oils, which makes it particularly suitable for treating stocks of a more highly paraffinic nature, such as from Mid-Continent stocks and Pennsylvania stocks. The 40 boiling point of the compound is 184° C., which 45 is sufficiently low to permit of its efficient removal from the oil.

The treatment of petroleum lubricant oil stock, containing both paraffinic and naphthenic constituents, with the solvent (benzylamine) 50 comprises intimately mixing the petroleum stock and the benzylamine. I have found that the benzylamine extracts or dissolves out naphthenic constituents from the petroleum stock undergoing treatment, and must be used in relative propor- 55

tion sufficient to effect the removal of such constituents. The benzylamine must be used in proportions sufficient to establish two liquid phases; viz., a solvent phase consisting mainly of benzylamine and containing the extracted naphthenic substances and an oily phase consisting mainly of the oil and containing some benzylamine. The extraction of the petroleum stock with the benzylamine, as just described, can be effected either in batch or continuous operation as desired. After the extraction is complete, the two phases, which consist of two superimposed liquid layers, are separated by drawing off the layers separately. Solvent may be recovered from the solvent layer by distillation and traces of solvent may be removed from the oily phase, as for instance by treatment with finely divided clay, to produce refined lubricating oil.

As an example of the efficacy of benzylamine as a refining agent for petroleum lubricating oil stock the following example is presented in which one volume of a dewaxed and deasphaltized residuum from Mid-Continent crude was treated at 20° F. with five volumes of benzylamine in a batch extraction. The comparative tests on the oil before and after treatment are as follows:

| 30                                                                            | Gravity,<br>°A. P. I. | S. U. V. |         | V. I. | Carbon<br>residue |
|-------------------------------------------------------------------------------|-----------------------|----------|---------|-------|-------------------|
|                                                                               |                       | 100° F.  | 210° F. |       |                   |
| Dewaxed and deasphalted residuum.                                             | 23.8                  | 1180     | 85.0    | 70    | 1.80              |
| Dewaxed and deasphalted residuum extracted with 5 vols. benzylamine at 20° F. | 27.8                  | 649      | 71.9    | 98    | 0.6               |

The above results indicate a very substantial improvement in viscosity index and carbon residue, and may be taken as typical of the capabilities of this solvent refining reagent on oils of a high paraffinic nature, as it will be noted that the oil treated had already been deasphaltized.

A satisfactory degree of improvement can be obtained ordinarily by treatment of one volume of oil with from one to seven and preferably from three to five volumes of benzylamine. The temperature of the solvent refining operation will ordinarily range from about 20° F. or 30° F. to 125° F., depending upon the stock which is treated, preferably between about 50° F. and 100° F.

I have found that benzylamine can readily and conveniently be employed to produce refined lubricating oils of especially high viscosity index as compared with the viscosity index which can readily be obtained by certain solvent refining agents of the prior art, for example, I have obtained by single batch extraction a dewaxed and deasphalted residuum from Mid-Continent crude with benzylamine a refined lubricating oil having a viscosity index of practically 100, while similar extraction of the same stock with many of the solvents commonly used commercially will produce refined oils of considerably lower viscosity indices. Also I have found that benzylamine is possessed of a relatively high solvent power which renders it capable of effective use on stocks in which the so-called "naphthenic" constituents of low viscosity index are present in relatively less amount.

As an example of the effectiveness of benzylamine when applied to stocks already highly paraffinic, I may cite the following example, in

which this solvent was applied to a Bradford long residuum:

Bradford (Pa.) long residuum

| Stock                                                          | Gravity<br>°A. P. I. | S. U. V.<br>210° F. | V. G. C. | Carbon<br>residue | 5  |
|----------------------------------------------------------------|----------------------|---------------------|----------|-------------------|----|
| Dewaxed residuum                                               | 27.4                 | 76.2                | 0.816    | 1.6               |    |
| Same after batch extraction with 5 vols. benzylamine at 80° F. | 29.1                 | 95.1                | 0.798    | 1.0               | 10 |

It is very evident from the above that benzylamine is well adapted to operations of the kind last discussed.

I claim:

1. The method of refining hydrocarbon lubricant oil stock to remove naphthenic substances therefrom which comprises the steps of mixing the oil stock with benzylamine, using a relative proportion of benzylamine sufficient to produce two liquid phases; viz., a solvent phase consisting mainly of benzylamine and an oily phase consisting mainly of the paraffinic part of oil and containing some benzylamine, removing the oily phase from the solvent phase, and removing the remainder of the benzylamine from the oily phase to obtain a refined lubricating oil.

2. The method of refining petroleum lubricant oil stock containing naphthenic substances which comprises extracting the said stock with liquid benzylamine to separate naphthenic substances therefrom, separating benzylamine and extracted matter from the said stock, and freeing the remaining oil of such benzylamine as it may contain to produce a refined lubricating oil.

3. The method of refining petroleum lubricant oil stock containing naphthenic constituents which comprises intimately mixing the oil stock with an agent comprising benzylamine in sufficient proportion relative to the stock to produce two phases, namely, a solvent phase consisting mainly of solvent and extracted naphthenic substances and an oily phase consisting mainly of the oil and containing some benzylamine, separating the two phases, and removing solvent from the oily phase to obtain a refined lubricating oil.

4. The method of refining petroleum lubricant oil stock to remove naphthenic constituents therefrom which comprises treating the petroleum stock with benzylamine at temperatures of from 20° F. to 125° F. and in the proportion of from one to seven volumes of benzylamine to one volume of stock, thereby producing two liquid phases, separating the respective phases, and removing the refined lubricating oil from the phase which contains same.

5. The method of refining petroleum lubricant oil stock containing naphthenic constituents to remove said naphthenic constituents therefrom which comprises the steps of intimately admixing the oil stock with benzylamine at a temperature of from 50° F. to 100° F. and in the relative proportions of from three to five volumes of benzylamine to one volume of oil sufficient to produce two liquid phases, namely a solvent phase consisting mainly of benzylamine and extracted naphthenic substances and an oily phase consisting mainly of the oil and containing benzylamine, removing the oily phase from the solvent phase, recovering benzylamine from the solvent phase and from the oily phase recovering lubricating oil having a viscosity index not substantially lower than the general order of 100 and a carbon residue not greater than 1.0.

6. A process for separating mineral oil con-

15

20

25

30

35

40

45

50

55

60

65

70

75

taining paraffinic and non-paraffinic fractions into more paraffinic and less paraffinic fractions which comprises commingling said oil with benzylamine to cause phase separation and separating the benzylamine and dissolved fractions from the remaining undissolved more paraffinic fractions.

7. A process for separating oil into fractions which comprises commingling said oil with benzylamine to cause separation of raffinate and extract phases, separating the extract phase containing benzylamine and oil fractions dissolved

therein from the raffinate phase containing the undissolved fractions and separating the benzylamine from said fractions.

8. A process for the separation of oil into fractions which comprises commingling said oil with benzylamine below the temperature of complete miscibility to cause separation of extract and raffinate phases, and separating the extract phase containing benzylamine and oil fractions dissolved therein from the raffinate phase containing the undissolved fractions.

THEODOR A. PETRY.